

1

2,822,234

ICE-COLORS IN TEXTILE PRINTING WITH  
NEUTRAL STEAM

Kurt Breig and Eugen Glietenberg, Leverkusen-Bayerwerk,  
Germany, assignors to Farbenfabriken Bayer Aktien-  
gesellschaft, Leverkusen, Germany, a corporation of  
Germany

No Drawing. Application December 16, 1954  
Serial No. 475,823

Claims priority, application Germany December 28, 1953

6 Claims. (Cl. 8—71)

The present invention relates to a process of preparing ice-colors in textile printing and dyeing.

In preparing ice-colors in textile printing from diazo-amino compounds, thickened caustic alkaline solutions of usual ice-color coupling components and alkali metal salts of diazoamino compounds containing solubilizing groups in the radical (stabilizer) not taking part in the formation of the dyestuff, are printed on the fibre and the dyestuff is developed by a treatment with dilute acid or, preferably, with acid-containing steam. This acid treatment involves a number of disadvantages and therefore many attempts have been made to effect the development of the ice-colors solely by applying neutral steam, especially since it is only possible by this kind of development to prepare ice-colors and vat-colors side by side. Thus very satisfactory results could be achieved by reducing the quantity of caustic alkali in the printing pastes or by adding compounds splitting off acid (cf. applications Nos. 313,582, now Patent No. 2,758,001, 313,583 and 390,084).

The ideal case would be, however, dyestuff combinations which can be developed in neutral steam without an addition of compounds splitting off acid or binding alkali. The solution of this problem would therefore mainly reside in the use of such diazoamino compounds which easily and completely split up in neutral steam but are completely stable in the cold and thereby afford a good keeping quality of the printing pastes. The capability of diazoamino compounds to split up greatly depends upon the basicity of the diazotizable amine on the one side and of the stabilizer on the other side. Every diazotized aromatic amine possesses, depending upon its substituents, a very different coupling energy and forms, according to whether it is more strongly or more weakly basic, diazoamino compounds which split up more easily or more difficultly. A similar statement holds true for the amines used as stabilizers. It is therefore necessary to adapt carefully to another amine and stabilizer if a quantitative scission of the diazoamino compound is to be obtained by applying solely neutral steam. The ideal case would be to provide the suitable stabilizer for each amine; this, however, would cause considerable additional costs when technically applied.

We have now found that the combinations of dihalogeno-alkyl- or dihalogeno-alkoxy anilines with 2-alkyl-amino-5(4)-sulfonylbenzoic acids represent ideal diazoamino compounds for the purpose discussed. They yield together with ice-color coupling components when developed with neutral steam very deep and strong prints on cellulosic fibres as well as a good fixation on staple fibre fabrics from regenerated cellulose. In spite of the easy scission in neutral steam the printing pastes exhibit a very good keeping quality. The prints further suffer no visible loss in depth of color if printed side by side with vat-colors. Also reducing agents and caustic alkali carried over from vat-color printing pastes have no detrimental influence upon the development of the dyestuffs.

2

It is important in this connection that the new combinations do not decrease in strength under the intermediate rollers in the composite print side by side with vat-colors; this means a special advance over the known combinations.

The combinations according to the present invention not only show very good properties in printing but also prints obtained therewith are distinguished by general good properties, in particular by an excellent fastness to light.

The following examples illustrate the invention without, however, limiting it thereto.

Example 1

15 1 mol of diazotized 1-amino-2-methyl-4,5-dichlorobenzene is slowly run, together with diluted sodium carbonate solution, into a weakly sodium carbonate alkaline solution of 1.1 mol of 2-ethylamino-5-sulfonylbenzoic acid, so that the solution shows a sodium carbonate alkaline reaction all the time. After stirring for 4 hours the coupling is complete, and the diazoamino compound can be salted out in crystalline form with sodium chloride.

20 60 grams of a mixture consisting of equivalent parts of the sodium salt of the diazoamino compound thus formed and the 1-(2',3'-hydroxynaphthoylamino)-2-ethoxy-benzene are dissolved in 50 ml. of alcohol or another suitable solvent and 15–20 grams of caustic soda solution of 38° Bé. in approximately 300 ml. of water and, after stirring into 500 grams of thickening agent, made up with water to 1000 grams. The printing paste thus obtained is printed on the fibre in customary manner.

25 After drying the printed textile material is steamed with neutral steam for about 5–10 minutes, whereby the development of the dyestuff takes place. After soaping at the boil and the usual removal of the thickening agent, the dyed textile is rinsed and dried. A clear scarlet is obtained which is very fast to light. The printing paste is of very good keeping quality. The depth of color of the printings on staple fibre fabric is equal to that of the

30 35 printings on cotton. In printing simultaneously with vat-dyestuffs, the combination shows on employing squeezing rollers no decline in the depth of color.

Example 2

40 45 When using according to Example 1 the sodium salt of the diazoamino compound prepared from 1-amino-2-methyl-4-bromo-5-chlorobenzene and the stabilizer employed in Example 1, together with the 1-(2'-hydroxy-carbazol-3'-carboylamino)-4-chlorobenzene, a full brown is obtained which is very fast to light.

Example 3

45 55 A printing paste prepared according to the preceding examples from the sodium salt of the diazoamino compound of 1-amino-3-methyl-4,6-dichlorobenzene with the stabilizer described in Example 1 and 1-acetoacetyl-amino-4-chloro-2,5-dimethoxybenzene yields on the fibre, after neutral development, a greenish yellow which is very fast to light.

60 65 Example 4

65 70 By replacing the sodium salt of the diazoamino compound of Example 1 by the sodium salt of the diazoamino compound from diazotized 1-amino-4-methyl-2,5-dichlorobenzene and 2-isopropylamino-5-sulfonylbenzoic acid as stabilizer, and using 1-(2',3'-hydroxynaphthoylamino)-2-methoxybenzene as coupling component, adding about 10–20 grams of caustic soda solution of 38° Bé. per kilogram printing color, a printing paste is obtained which yields on the fibre, after neutral steaming, a strong fast red, the depth of which on cotton is equal to that on staple fibre fabric.

## Example 5

1 mol of diazotized 1-amino-2-methoxy-4,5-dichlorobenzene is run into a sodium carbonate alkaline solution of 1.1 mol of the disodium salt of the 2-methylamino-5-sulfobenzoic acid, and the diazoamino compound thus formed is salted out with sodium chloride after its complete formation.

60 grams of a mixture consisting of equivalent parts of the sodium salt of the diazoamino compound thus formed and the 1-(2',3'-hydroxynaphthoyl-amino)-2-methoxybenzene are dissolved in about 50 ml. of glycol monoethyl ether or another suitable solvent and 10-20 grams of caustic soda solution of 38° Bé. in approximately 300 ml. of hot water and, after stirring into 500 grams of thickening agent, made up with water to 1000 grams. This printing paste yields, after neutral steaming, a full bluish red of excellent fastness to light. The depth of color on staple fibre fabric is in strength equal to that on cotton.

## Example 6

The sodium salt of the diazoamino compound of diazotized 1-amino-2-methoxy-4-bromo-5-chlorobenzene and the 2-ethylamino-5-sulfobenzoic acid as stabilizer yields in equivalent mixture with 1-benzoylacetylamin-4-benzoylamin-2,5-dimethoxybenzene under the conditions of Example 5, after steaming in neutral steam, a clear yellow which is very fast to light. The strength of color on cotton as well as on staple fibre fabric is equally deep.

We claim:

1. A process for printing textile fibres of the group consisting of cotton and regenerated cellulose fibers with insoluble azo dyestuffs developed on the fibre which comprises diazotizing a compound selected from the group consisting of dihalogeno-alkyl-anilines and dihalogeno-alkoxy-anilines, reacting the diazo compound formed with a compound selected from the group consisting of 2-alkylamino-5-sulfobenzoic acid and 2-alkylamino-4-sulfobenzoic acid in the presence of a fixed alkali to form an alkali salt of a diazoamino compound, mixing said alkali salt with an alkali salt of a coupling component, adding a thickener to the mixture, applying the resulting mixture to a textile fibre, and developing the dyestuff on said fibre by steaming with neutral steam.

2. A process for printing textile fibers of the group consisting of cotton and regenerated cellulose fibers with insoluble azo dyestuffs developed on the fiber which comprises diazotizing 1-amino-2-methyl-4,5-dichlorobenzene, reacting the diazo compound formed with 2-ethylamino-5-sulfobenzoic acid in the presence of a fixed alkali to form an alkali salt of a diazoamino compound, mixing said alkali salt with an alkali salt of 1-(2',3'-hydroxynaphthoyl-amino)-2-methoxybenzene, adding a thickener to the mixture, applying the resulting mixture to a textile fiber, and developing the dyestuff on said fiber by steaming with a neutral steam.

3. A process for printing fibers of the group consisting of cotton and regenerated cellulose fibers with insoluble azo dyestuffs developed on the fiber which comprises diazotizing 1-amino-3-methyl-4,6-dichlorobenzene, reacting the diazo compound formed with 2-ethylamino-5-sulfobenzoic acid in the presence of a fixed alkali to form

an alkali salt of a diazoamino compound, mixing said alkali salt with an alkali salt of 1-acetylacetamino-4-chloro-2,5-dimethoxybenzene, adding a thickener to the mixture, applying the resulting mixture to a textile fiber, and developing the dyestuff on said fiber by steaming with a neutral steam.

4. A process for printing textile fibers of the group consisting of cotton and regenerated cellulose fibers with insoluble azo dyestuffs developed on the fiber which comprises diazotizing 1-amino-2-methyl-4-bromo-5-chlorobenzene, reacting the diazo compound with 2-ethylamino-5-sulfobenzoic acid in the presence of a fixed alkali to form an alkali salt of a diazoamino compound, mixing said alkali salt with an alkali salt of 1-(2'-hydroxycarbazol-3'-carboylamino)-4-chlorobenzene, adding a thickener to the mixture, applying the resulting mixture to a textile fiber, and developing the dyestuff on said fiber by steaming with a neutral steam.

5. A process for printing textile fibers of the group consisting of cotton and regenerated cellulose fibers with insoluble azo dyestuffs developed on the fiber which comprises diazotizing 1-amino-4-methyl-2,5-dichlorobenzene, reacting the diazo compound with 2-isopropylamino-5-sulfobenzoic acid in the presence of a fixed alkali to form an alkali salt of a diazoamino compound, mixing said alkali salt with an alkali salt of 1-(2',3'-hydroxynaphthoyl-amino)-2-methoxybenzene, adding a thickener to the mixture; applying the resulting mixture to a textile fiber, and developing the dyestuff on said fiber by steaming with a neutral steam.

6. A process for printing textile fibers of the group consisting of cotton and regenerated cellulose fibers with insoluble azo dyestuffs developed on the fiber which comprises diazotizing 1-amino-2-methoxy-4,5-dichlorobenzene, reacting the diazo compound with 2-methylamino-5-sulfobenzoic acid in the presence of a fixed alkali to form an alkali salt of a diazoamino compound, mixing said alkali salt with an alkali salt of 1-(2',3'-hydroxynaphthoyl-amino)-2-methoxybenzene, adding a thickener to the mixture, applying the resulting mixture to a textile fiber, and developing the dyestuff on said fiber by steaming with a neutral steam.

## References Cited in the file of this patent

## UNITED STATES PATENTS

|           |             |                |
|-----------|-------------|----------------|
| 1,882,561 | Haller      | Oct. 11, 1932  |
| 2,093,402 | Dahlen      | Sept. 21, 1937 |
| 2,338,639 | Heaton      | Jan. 4, 1944   |
| 2,396,357 | Wiest       | Mar. 12, 1946  |
| 2,522,838 | Petitcolas  | Sept. 9, 1950  |
| 2,675,374 | Petitcolas  | Apr. 13, 1954  |
| 2,758,001 | Glietenberg | Aug. 7, 1956   |

## FOREIGN PATENTS

|           |               |               |
|-----------|---------------|---------------|
| 497,407   | Great Britain | Dec. 19, 1938 |
| 1,042,356 | France        | June 3, 1953  |
| 1,056,504 | France        | Oct. 21, 1953 |

## OTHER REFERENCES

"Chem. Technology of Dyeing and Printing," by L. Diserens, translated by Wengraf and Baumann, vol. 4, pp. 304, 305, 316; published in N. Y. C. by Reinhold Corp., 1948.